

H. J. & A. PHILLIPS.  
MANUFACTURE OF COAL BRIQUETS.  
APPLICATION FILED JAN. 31, 1914.

1,149,536.

Patented Aug. 10, 1915.



### *Witnesses.*

J. B. Bluming  
Jesse B. Heller

## *Inventors.*

H. J. Phillips  
Arthur Phillips  
by Baker, Byrnes & Farmer  
Attys.

# UNITED STATES PATENT OFFICE.

HENRY JOSHUA PHILLIPS, OF LONDON; AND ARTHUR PHILLIPS, OF TREDEGAR, ENGLAND, ASSIGNEES TO PURE COAL BRIQUETTES LIMITED, OF CARDIFF, WALES.

## MANUFACTURE OF COAL BRIQUETS.

1,149,536.

Specification of Letters Patent. Patented Aug. 10, 1915.

Application filed January 31, 1914. Serial No. 815,688.

*To all whom it may concern:*

Be it known that we, HENRY JOSHUA PHILLIPS and ARTHUR PHILLIPS, subjects of the King of England, residing in London, England, and Tredegar, county of Monmouth, England, respectively, have invented certain new and useful Improvements in the Manufacture of Coal Briquets, of which the following is a specification.

10 This invention relates to a new and improved method of manufacturing coal briquets, whereby we are enabled to cheaply produce non-porous and weather-proof briquets from small coal, without the use 15 of a binding agent.

The process may be carried out by any well known apparatus in the following manner: (a) grinding the coal with water to a pulp; (b) feeding this pulp directly and 20 without allowing the pulp to settle and stratify to a mold and compressing it therein to eliminate a large proportion of the water and consolidate the pulp into briquet form; (c) passing the partially-formed 25 briquets through a tunnel wherein the temperature gradually increases from a temperature at the entrance substantially below the boiling point of water to a temperature at the exit approximating to but below the decomposing point of the coal used for the briquets, and then (d) subjecting the briquets thus dried and incipiently softened to a hot and relatively high compression to complete 30 the consolidation thereof.

35 The temperatures and pressures at which it is preferred to work are indicated particularly hereinafter, and there is also described in detail a construction of mold and plungers which may be used in connection with 40 step (b) above.

For a more complete understanding of the invention reference is directed to the accompanying drawings wherein a particular construction of mold and plungers is illustrated 45 for compressing the wet pulp from which the briquets are made.

In these drawings—Figure 1 is a vertical section on the line 1—1 of Fig. 2, and Fig. 2 is a plan.

50 Like letters of reference refer to like parts throughout the drawings.

In carrying out the invention the small coal to be converted into briquets is first ground in hot or cold water to a pulp in any 55 suitable pug, tube or other mill to any suit-

able degree of fineness. 100 parts by weight of coal to 45–60 parts by weight of water will be found to be a suitable proportion. The aqueous pulp produced is then fed directly, *i. e.* without being left to settle, into 60 a mold wherein it is compressed to eliminate a large proportion of the water and consolidate it into briquet form. Three to five tons per square inch will be found to be a convenient pressure, and this will produce 65 cohesive but damp briquets.

In order to obviate the necessity for allowing the pulp to settle and a certain proportion of the water to drain away, which operation is rather lengthy, and gives rise 70 moreover to stratification, so that possibly the briquets might be produced with varying proportions of the different grades or meshes of coal (should such be present), the pulp is preferably fed to the mold and plungers shown in the drawings. The construction shown is specially adapted for permitting the water contained in the pulp to drain away readily when pressure is applied to the 75 pulp by means of the plungers.

The mold shown in the drawings comprises an outer casing A of rectangular section. This casing is lined on the interior with a series of vertical bars which are secured to the casing by bolts passed through flanges B' on the bars and flanges A' on the casing. The flanges A' on the casing have grooves sunk therein to receive the flanges B' so that the end surfaces of the mold may be unbroken. The adjacent side faces of 80 the bars, *i. e.* the faces B<sup>2</sup>, B<sup>3</sup>, converge and meet at the edges B<sup>4</sup> situated at the interior of the mold. Thus at the interior of the mold the bars form practically continuous surfaces, but at the back of each of these surfaces there runs a series of vertical throughways of V-section which can convey away 85 any water forced out of the pulp and between the bars. At the corners of the casing A filling bars B<sup>5</sup> are provided to operate in conjunction with the bars B.

Mounted to reciprocate within the mold there are shown two oppositely-acting plungers C, D which are fluted on their vertical faces at C' and D' respectively and on their 90 end faces at C<sup>2</sup> and D<sup>2</sup> respectively. The plungers are also each provided on their end faces with a series of bars C<sup>3</sup> and D<sup>3</sup>. These bars run transversely of the flutes C<sup>2</sup> and D<sup>2</sup> in the end faces of the plungers, and 105 110

the bars are secured to the plungers by screws C<sup>4</sup> and D<sup>4</sup>. The adjacent side faces of the bars C<sup>3</sup> and D<sup>3</sup> converge in a similar manner to the faces B<sup>2</sup> and B<sup>3</sup> of the bars 5 B, and meet at the edges C<sup>5</sup> and D<sup>5</sup> which are situated at the interior of the mold. It is thus provided that water pressed out of the pulp may readily drain away from the faces of the plungers through the flutes and 10 throughways provided.

Conveniently the bars B, B<sup>5</sup>, C<sup>3</sup> and D<sup>3</sup> are of some non-rusting metal, such as phosphor-bronze.

The construction of the above described 15 mold and plungers is claimed in copending application, Serial No. 850,414, filed July 11, 1914:

The damp blocks or briquets made in the 20 mold above described are placed on trolleys or endless belts or the like and carried by them through a differentially-heated tunnel, wherein the temperature gradually increases from the entrance to the exit.

The temperature at the entrance of the 25 tunnel should be substantially below the boiling point of water. 80° C. is a suitable temperature. With this temperature at the entrance any water present in the briquets will be gradually (not suddenly) converted 30 into steam. This is an important point, since if the temperature were 100° C. or higher the water in the briquets would be immediately converted into steam and would probably crack the briquets in escaping therefrom.

The temperature at the exit of the tunnel approximates to but is below the decomposing point of the coal used for the briquets. With certain kinds of anthracite coal the 40 temperature may be as much as 500° C. but with bituminous coal the temperature must not exceed say 300° C. It must be borne in mind that the heating in the tunnel of the briquets after they have 45 been dried, is only to be carried so far as to cause an incipient softening of the coal; the decomposing point of the coal is not to be reached. For an ordinary sample of semi-bituminous coal 250° C. will be found 50 to be a suitable temperature for the exit of the tunnel, and therefore for the maximum temperature to which the coal is heated.

The dried and incipiently softened briquets issuing from the tunnel are placed in 55 a second mold and subjected to a hot and relatively high compression to complete the consolidation of the briquets. The molds are of similar shape to those shown in the drawings but may be plain, i. e. not provided with the drainage arrangements shown in the drawings. The molds for the 60 second compression should be of fractionally larger dimensions than the molds used for the first compression as the briquets will 65 be found to have swelled slightly owing to

the heating. The mold for the second compression may be kept hot by super-heated steam in any convenient manner. The pressure is preferably applied simultaneously at both ends of the mold and the degree of 70 pressure varies according to the class of coal used; 5-15 tons per square inch will be found to be a suitable range of pressures.

It will be appreciated that different classes 75 of small coals require different degrees of pressure and temperature for their manufacture into briquets. The degrees of temperature and pressure will be readily found by experiment, but it will be found that the particulars given herein cover all average 80 cases.

It will be seen that according to the present invention coal briquets are manufactured without the addition of a binding agent. If 85 a binding agent can be found which will stand both the effects of the temperature to which the coal is subjected according to the process above described and the effects of wet after the briquets are finished, then it may be thought advisable in some cases to 90 include a percentage of this binding agent with the coal. The addition of a binding agent is not essential however; as by following the instructions given excellent pure-coal briquets can be manufactured. 95

The invention is not limited to the employment of the precise construction of mold and plungers hereinbefore described. These will give good results but any other construction may be substituted if found desirable. 100

What we claim as our invention and desire to secure by Letters Patent is:—

1. The method of making coal briquets which comprises grinding coal to a pulp in 105 the presence of water, then feeding the pulp to a mold without allowing the pulp to settle and stratify, then compressing the pulp in the mold to eliminate a large proportion of water and compress the pulp into briquet 110 form, then passing the partially-formed briquet into a heating chamber and gradually increasing the temperature therein from a temperature below the boiling point of water to a temperature slightly below the 115 temperature at which the coal will decompose, and then subjecting the dried and incipiently softened briquet to a hot and relatively high compression to complete the consolidation thereof. 120

2. The method of making coal briquets which comprises grinding about 100 parts by weight of coal in the presence of 45 to 60 parts of water by weight, then feeding the pulp to a mold, then compressing the 125 pulp in the mold to eliminate a large proportion of the water and consolidate the pulp into briquet form, then passing the partially formed briquet through a heating chamber and during its passage there- 130

through heating said briquet to a temperature slightly below the temperature at which the coal will decompose, and then subjecting the briquet thus dried and incipiently softened to a hot and relatively high compression to complete the consolidation thereof.

3. The method of making coal briquets which comprises grinding 100 parts by weight of coal in the presence of 45 to 60 parts of water by weight, then feeding the pulp to a mold without allowing the pulp to settle and stratify, then compressing the pulp in a mold to eliminate a large proportion of water and compressing the pulp into briquet form, then passing the partially-formed briquet through a heating chamber and during its passage therethrough heating said briquet to a temperature slightly below the temperature at which the coal will decompose, and then subjecting the briquets thus dried and incipiently softened to a hot and relatively high compression to complete the consolidation thereof.

4. The method of making coal briquets which comprises grinding coal to a pulp in the presence of water, then feeding the pulp to a mold, then compressing the pulp in the mold to eliminate a large proportion of the water and compressing the pulp into briquet form, then passing the partially-formed briquet through a heating chamber and during its passage therethrough heating said briquet to a temperature of 200° centigrade to 500° centigrade, and then subjecting the briquet thus dried and incipiently softened to a hot and relatively high compression to complete the consolidation thereof.

5. The method of making coal briquets which comprises grinding 100 parts by weight of coal in the presence of 45 to 60 parts by weight of water, then feeding the pulp to a mold, then compressing the pulp in the mold to eliminate a large proportion of water and compressing the pulp into briquet form, then passing the partially-formed briquet through a heating chamber and during its passage therethrough heating said briquet to a temperature of 200° centigrade to 500° centigrade, and then subjecting the briquet thus dried and incipiently softened to a hot and relatively high compression to complete the consolidation thereof.

6. The method of making coal briquets which comprises grinding 100 parts by weight of coal in the presence of 45 to 60 parts by weight of water, then feeding the pulp to a mold and subjecting it to a pressure of 3 to 5 tons per square inch within the mold to eliminate a large proportion of the water and compress the pulp into briquet form, then passing the partially-formed briquet into a heating chamber and gradually increasing the temperature there-

in from a temperature below the boiling point of water to a temperature slightly below the temperature at which the coal will decompose, and then subjecting the dried and incipiently softened briquet to a pressure of 5 to 15 tons per square inch in a mold heated by superheated steam to complete the consolidation of the briquet.

7. The method of making coal briquets which comprises grinding about 100 parts by weight of coal in the presence of 45 to 60 parts by weight of water, then feeding the pulp to a mold and subjecting it therein to a pressure of 3 to 5 tons per square inch to eliminate a large proportion of the water and compress the pulp into briquet form, then passing the partially-formed briquet through a heating chamber and during its passage therethrough heating said briquet to a temperature of 200° centigrade to 500° centigrade, and then subjecting the briquet thus dried and incipiently softened to a pressure of 5 to 15 tons per square inch in a mold heated by superheated steam to complete the consolidation of the briquet.

8. The method of making coal briquets which comprises grinding about 100 parts by weight of coal in the presence of 45 to 60 parts by weight of water, then feeding the pulp to a mold and subjecting it therein to a pressure of 3 to 5 tons per square inch to eliminate a large proportion of the water and compress the pulp into briquet form, then passing the partially-formed briquet into a heating chamber and gradually increasing the temperature thereof from 80° centigrade to 250° centigrade to 500° centigrade, and then subjecting the briquet thus dried and incipiently softened to a pressure of 5 to 15 tons per square inch in a mold heated by superheated steam to complete the consolidation of the briquet.

9. The method of making coal briquets which comprises grinding in the proportion of 100 parts of coal by weight in the presence of 45 to 60 parts by weight of water, then feeding the pulp directly to a mold having two oppositely acting plungers and subjecting it therein to a pressure of 3 to 5 tons per square inch to eliminate a large proportion of the water and compress the pulp into briquet form, then passing the partially-formed briquet through a heating chamber wherein the temperature gradually increases from 80° centigrade at the entrance to 250° centigrade to 500° centigrade at the exit according to the quality of the coal used for the briquets, then subjecting the briquets thus dried and incipiently softened to a pressure of 5 to 15 tons per square inch in the mold heated by superheated steam and in which the briquet is acted upon by plungers moving in opposite directions to consolidate the briquet.

10. The method of making coal briquets

which comprises grinding in the proportion of 100 parts of coal by weight in the presence of 45 to 60 parts by weight of water, then feeding the pulp to a mold without allowing the pulp to settle and stratify and compressing it therein with two oppositely acting plungers under a pressure of 3 to 5 tons per square inch to eliminate a large proportion of the water and compress the pulp into briquet form, then passing the partially-formed briquet through a heating chamber wherein the temperature gradually increases from 80° centigrade at the entrance to 250° centigrade to 500° centigrade at the exit according to the quality of the

coal used for the briquet, then subjecting the briquet thus dried and incipiently softened to a pressure of 5 to 15 tons per square inch in a mold heated by superheated steam and in which the briquet is acted upon by 20 plungers moving in opposite directions to consolidate the briquet.

In testimony whereof we have signed our names to this specification in the presence of two subscribing witnesses.

HENRY JOSHUA PHILLIPS.  
ARTHUR PHILLIPS.

Witnesses:

NORMAN M. INGLEDINE,  
GODFREY W. JONES.